

## UNITED STATES PATENT OFFICE.

CHARLES TYNDALE EVANS, OF TITUSVILLE, PENNSYLVANIA.

## ALLOY STEEL AND PROCESS OF MAKING THE SAME.

No Drawing.

Application filed April 3, 1922. Serial No. 549,210.

*To all whom it may concern:*

Be it known that I, CHARLES TYNDALE EVANS, a citizen of the United States, residing at Titusville, county of Crawford, and State of Pennsylvania, have invented certain new and useful Improvements in Alloy Steels and Processes of Making the Same, fully described and represented in the following specification.

10 This invention relates to improvements in alloy steels, particularly steels adapted for cutlery, and also relates to improvements in processes for making such steels.

The main object of the invention is to provide a steel which, when worked into the desired article as, for example, by forging at the proper temperature and properly hardened, will be substantially non-corrosive under the conditions to which such steel articles are subjected, while at the same time having all the valuable properties of the best cutlery steels.

A further object of the invention is to provide a process which may be readily carried out for the manufacture of the alloy steels constituting a part of this invention.

The product included in this invention comprises an alloy steel of the composition described hereinafter and pointed out in the claims, and the process comprises the steps which will first be fully described and then set forth in the claims.

The alloy steel which represents the best embodiment of the invention consists of the following:

|             | Per cent. |
|-------------|-----------|
| Iron        | 83.9      |
| Carbon      | 0.6       |
| Chromium    | 7.0       |
| 40 Tungsten | 7.0       |
| Silicon     | 1.0       |
| Manganese   | 0.5       |
| Phosphorus  | 0.0       |
| Sulphur     | 0.0       |

45 The above represents what might be called an ideal alloy for the purposes of the invention. In practice, it is not always possible to produce material having the analysis stated above. For example, it is rarely possible to have the alloy entirely free from phosphorus or sulphur. It is very important, however, to keep these ingredients as low as possible.

In carrying out the invention in practice

following the above formula the alloy steels produced have varied somewhat in composition. The following formula will include a number of such alloy steels which have been made and tested and found to be eminently satisfactory for the purposes of this invention:

|            | Per cent.      |
|------------|----------------|
| Carbon     | 0.500 to 0.850 |
| Chromium   | 6.770 to 7.530 |
| Tungsten   | 6.36 to 8.080  |
| Silicon    | 0.810 to 1.130 |
| Manganese  | 0.500 to 0.700 |
| Phosphorus | about .012     |
| Sulphur    | about .018     |

The principal remaining ingredient is iron.

Alloy steels of substantially the composition stated above have been worked into cutlery and have given results much superior to those obtained with chromium alloy steels heretofore known.

These new steels are readily worked, but when being hardened they should be heated to somewhat higher temperatures than are used when working common cutlery steels. Highly satisfactory results are obtained if the present steels are hardened at a temperature of about 2000° F. While they can be hardened satisfactorily if heated to a temperature as low as about 1900° F. the desired results are obtained with greater ease and certainty if the heating be carried to about 2100° F.

The duration of the heat treatment is also of some importance, because the advantageous properties of the material are best developed by what may be termed a thorough soaking heat. While the length of time varies according to size of the material which is being worked, and therefore cannot well be stated in minutes, it suffices for those skilled in the art of steel treatment to say that the steel alloy of the present invention should remain in the heating furnace at about 2000° F. for a somewhat longer time than is ordinarily considered necessary for a good high carbon cutlery steel.

It has been found that an alloy steel of the type set forth above, worked in the usual manner, and hardened by the methods described, gave cutlery articles of greatly improved properties. Not only was a fine cut-

lery edge obtained, but this edge was capable of withstanding hard usage, that is to say, was maintained as well as with the very best high carbon cutlery steels. Furthermore, the material had a high resistance to a permanent set, and was relatively tough as compared with the prior steels high in chromium.

A further important advantage of these 10 alloy steels is that after the heat treatment referred to above, they are non-corrosive under the normal conditions to which articles of cutlery are subjected. For example, a polished surface of the finished article will 15 not rust or stain by the action of the air, the usual organic acids, weak inorganic acids, alkalies, salt water or the like.

Owing to the hard close texture which 20 may be given to this steel by treatment as described, it may be polished to a mirror surface and will retain such a polish indefinitely, so that the material seems to make 25 possible a great advance in the mirror art.

It is to be understood, however, that this 25 property of non-corrodibility is only developed by the heat treatment hereinbefore described. Prior to this treatment the alloy steel is corrodible. Furthermore, the non-corrosive property of the alloy steel when 30 developed by the heat treatment and working is not confined merely to the surface of the material but seems to extend throughout the mass. This is important in cutlery articles because subsequent grinding does not 35 lead to a corrodible surface.

In carrying out the process for the manufacture of the new product hereinbefore referred to, the starting materials or mix may be as follows:

|                  | Parts.     |
|------------------|------------|
| Iron             | 707.50     |
| Ferro-chromium   | 104.40     |
| Tungsten powder  | 63.75      |
| Manganese        | 6.25       |
| Silico-zirconium | 13.75      |
| Ferro-silicon    | 4.35       |
| <br>Total        | <br>900.00 |

This mix is melted in the usual way, for 50 example, as in the manufacture of crucible steel. It may then be cast into ingot form and worked down by the usual methods of working crucible steel. The bars or rods are cut to lengths suitable for the articles 55 which it is desired to produce, and these blanks are heated and forged into the desired shapes. Finally the material is hardened in the manner hereinbefore described and may be finished by tempering and polishing in the usual way. The particular 60 point to which attention is called in connection with the above process is that the starting material comprises a zirconium compound, in this case silico-zirconium, yet the 65 resultant product, viz., the alloy steel, when

analyzed by the usual methods of analysis employed in the steel works, does not seem to show the presence of any zirconium. It may be possible that by some very refined methods of analysis some zirconium or zirconium compounds might be detected in the alloy steel. It may be, however, that the zirconium compound merely performs the function of a scavenging material or deoxidizer in making the original ingot, and hence does not appear in the alloy steel product. While the presence of zirconium in the mix seems to be important in that with it the desired alloy steel may be produced with certainty, apparently the presence of zirconium in the alloy steel, if any is present there, is not controlling. This seems to be shown by the fact that substantially the same alloy steel having substantially the same desirable properties as hereinbefore 80 pointed out has been produced by a modification of the above process in which the starting material was as follows:

|                 | Parts. | 90 |
|-----------------|--------|----|
| Iron            | 790    | 90 |
| Ferro-chromium  | 105    |    |
| Tungsten powder | 75     |    |
| Manganese       | 4      |    |
| Ferro-silicon   | 26     |    |

Using this starting mixture, melting it, 95 casting it into an ingot, working it down to blanks, and making the cutlery articles from such blanks by the same steps as hereinbefore described, resulted in articles having all the desirable properties which it is the object of this invention to attain and yet, obviously the alloy steel so produced could not have any zirconium in it. By both processes the alloy steel product will give an analysis showing the same ingredients 100 set forth on page 2 of this specification and in proportions falling within the limits there stated. It is to be noted, however, that the process carried out with the mixture containing silico-zirconium seems to be 110 more reliable than the modified process given above where the silico-zirconium is omitted from the mixture.

Variations may be made in the composition of the alloy steel and in the process 115 without departing from the invention. For example, the carbon content may be increased to some extent, for example, up to about 1 per cent, thereby giving a harder steel, but in such case more care will be required in working the steel into finished articles. Where the carbon content is kept at about the higher limit of .85 shown in the table, page 2, it will be found that the temperature for hardening may be kept 120 regularly at about 1900° F., whereas with a lower carbon content this hardening temperature is best kept at about 2000°. Where the mix is made with the usual commercial ferro-chromium such as is used in making 125

high-speed steels, the carbon content will run toward the higher limit given in the table. If it is desired to keep the carbon near the low limit, the mix should be made with a ferro-chromium lower in carbon or with the so-called "carbon-free" ferro-chromium.

By somewhat reducing the silicon content while increasing the carbon content to a reasonable extent, the quality of the product and the ease of working it will not be affected injuriously, and at the same time the hardening temperatures may be kept down to around 1900° F. With low carbon content, the silicon may go as high as about 2.0 per cent.

Furthermore, an alloy steel which will develop fully the desired non-corrosive properties, when hardened at the lower temperature of around 1900°, may be obtained by the addition of nickel. While the amount of nickel used may vary, I have found that 3½ per cent is about as high as is necessary. When more than this amount is used there is always a danger of segregation of the nickel in the finished articles, and this may give a bad appearance to the polished article, and, possibly, may lead to some corrodibility.

As illustrating the use of nickel in the alloy steels of this invention, I submit the following examples in which first is stated the mixture to be melted and then the analysis showing the essential ingredients of the respective alloy steels, viz.:

*Mix.*

|                  | Parts. |
|------------------|--------|
| Iron             | 725    |
| Ferro-chromium   | 105    |
| Tungsten, powder | 75     |
| Ferro-silicon    | 20     |
| Nickel           | 25     |
| Nickel-zirconium | 50     |
| Manganese        | 5      |

*Analysis.*

|           | Per cent. |
|-----------|-----------|
| Carbon    | 0.618     |
| Chromium  | 7.83      |
| Tungsten  | 6.56      |
| Manganese | 0.61      |
| Silicon   | 1.15      |
| Nickel    | 3.28      |

The principal remaining ingredient is iron.

*Mix.*

|                  | Parts. |
|------------------|--------|
| Iron             | 725    |
| Ferro-chromium   | 105    |
| Tungsten, powder | 75     |
| Ferro-silicon    | 20     |
| Nickel           | 25     |
| Nickel-zirconium | 50     |
| Manganese        | 5      |

*Analysis.*

|           | Per cent. |
|-----------|-----------|
| Carbon    | 0.486     |
| Chromium  | 7.58      |
| Tungsten  | 6.26      |
| Manganese | 0.73      |
| Silicon   | 1.09      |
| Nickel    | 3.46      |

The principal remaining ingredient is iron.

These nickel-containing alloys gave very satisfactory results.

It is to be noted that in the first example of the product set forth on page 1 of this specification, the tungsten content is specified around 7 per cent. I have found that more tungsten may be employed if desired. However, it is ordinarily not necessary to go above 10 per cent tungsten, because tungsten is an expensive material, yet sometimes it may be desirable to increase the percentage of it in order to get somewhat harder steels. If, however, the tungsten is to be increased above 10% it becomes important to cut down the silicon content of the alloy steel.

While in connection with the process I have described the use of zirconium in the mixture serving as a starting material, I may use in place thereof cerium, or titanium. In using these equivalents of the zirconium, they may be employed commercially in the form of the ferro-alloys.

The manganese content of the alloy may sometimes be as low as .25%, particularly when the toughness of the resultant product is not important or where the iron used in making the mix is very pure. On the other hand, if copper is present as an impurity in the starting materials, which sometimes happens with certain irons, it may be well to run the manganese content of the alloy steel as high as .75%. The manganese seems to have the property of neutralizing any bad effects of the copper. My experience indicates that the manganese content has an effect in determining the toughness of the finished product. However, I find no advantage in using more than the high limit hereinbefore stated.

The chromium content may be reduced somewhat below the minimum limit stated in the formula on page 2 without materially departing from the qualities of the finished product. For example, the chromium content may be as low as 6%.

A steel containing less than 7% of tungsten will be satisfactory for some purposes where the cutting edge is not subjected to a very severe usage as, for example, with fruit knives or the like. In this case the tungsten content may be reduced as low as 4% in the alloy steel, but, as before indicated, with a slight loss in the durability of the cutting edge.

## What is claimed is:

1. A ferrous alloy having a carbon content of not more than about 1%, a chromium content of not less than 6% and not more than about 7.53%, and a tungsten content of more than about 4%.
2. A ferrous alloy having a carbon content of not more than about 1%, a chromium content of not less than 6% and not more than about 7.53%, a tungsten content of more than about 4%, and a manganese content of .25 to .75%.
3. A ferrous alloy having a carbon content of not more than about 1%, a chromium content of not less than 6% and not more than about 7.53%, a silicon content of essential amount but not more than 2%, and a hardening ingredient such as tungsten not exceeding 10%.
4. A ferrous alloy substantially free from phosphorus and sulphur and having a carbon content of between .5 and .85%, a chromium content of about 6 to 7.53%, a tungsten content of more than 6%, a silicon content of essential amount but less than 2%, and a manganese content of about .5 to .7%.
5. A ferrous alloy having a carbon content of not more than about 1%, a chromium content of not less than 6% and not more than about 7.53%, a hardening ingredient such as tungsten not exceeding 10%, and which, when hardened at a sufficiently high temperature, develops the property of non-corrosiveness, substantially as described.
6. The process of making a non-corrosive, wrought ferrous article, which consists in mixing the ingredients to give the desired percentages of iron, chromium, tungsten, manganese and silicon in the finished article, together with zirconium, cerium or titanium, then melting the mixture, working it into the desired article and hardening at a temperature high enough to develop the non-corrosive properties, substantially as described.
7. A ferrous alloy substantially free from phosphorus and sulphur and having a carbon content of between .5 and .85%, a chromium content of about 6 to 7.53%, a tungsten content of more than 6%, a silicon content of less than 2%, a manganese content of about .5 to .7%, and nickel in substantial amount but not more than 3½%.
8. The process of making a non-corrosive, wrought ferrous article, which consists in mixing the ingredients to give the desired percentages of iron, nickel, chromium, tungsten, manganese and silicon in the finished article, together with zirconium, cerium or titanium, then melting the mixture, working it into the desired article and hardening at a temperature high enough to develop the non-corrosive properties substantially as described.

In testimony whereof, I have hereunto set my hand.

CHARLES TYNDALE EVANS.